

2,867,533

METHOD FOR OVERCOMING EMBRITTLEMENT  
OF STEEL ALLOYSLeroy E. Fink, Beaverton, Oreg., assignor to Electric  
Steel Foundry Company, Portland, Oreg., a corpora-  
tion of OregonNo Drawing. Application September 23, 1957  
Serial No. 685,415

2 Claims. (Cl. 75—130.5)

This invention relates to a method for overcoming embrittlement of steel alloys, and is particularly useful in combating the embrittlement or cracking tendency known as "hot shortness" in austenitic stainless cast steels.

This application is a continuation-in-part of my co-pending applications, Serial No. 477,576, filed December 27, 1954, now Patent No. 2,811,438, and Serial No. 485,341, filed January 31, 1955, now abandoned.

In the manufacture of austenitic stainless steels, it is found that the alloys are difficult to case, weld, or hot work, without the tendency to be "hot short." "Hot shortness" may be defined as a brittleness which occurs in the metal when hot, the metal separating in most cases at the grain boundary. In the casting operation, as the casting cools from the liquid state to the solid state in the mold, the mold sets up a restriction to the contracting metal. Many steels and alloys are strong enough to resist this restriction, but considerable difficulty is found with austenitic stainless steels, and tearing occurs in the casting, which must be welded. Welding also becomes a problem, since the metal adjacent the weld is heated, and frequently cracking will occur in this adjoining portion, requiring continual repairs, and eventually the product must be scrapped.

I have discovered that such austenitic stainless steel alloys may be effectively treated to prevent "hot shortness" by adding to the alloy while molten a compound of vanadium, titanium and boron. I prefer to add the vanadium and titanium as ferro-compounds, and I find it desirable to employ the vanadium and titanium as a combined ferro-compound. The combination of vanadium and titanium in a ferro-compound by molten agglomeration is well known in the art, and a detailed description herein is believed unnecessary.

The combination of vanadium, titanium and boron may be added to the molten alloy while in the furnace, as, for example, in an arc or induction electric furnace, just before tapping. If desired, it may be added to the ladle during tapping.

The proportions of the compounds are employed within certain limits which are effective in producing the best results. For example, the vanadium is satisfactorily used in the proportion of 0.02% to 1.07%, the titanium in the proportion of 0.01% to 0.6%, while the boron is added in a very small amount, ranging from a trace to 0.002%. I have found that best results are obtained when the vanadium is used in the range of 0.05% to 0.25%, the titanium in the range of 0.01% to 0.15%, and the boron in about 0.002%.

In general, the vanadium employed is about twice that of the titanium, although I find that best results are obtained when the titanium is about three-fifths of the vanadium. I find that all three materials, namely, the vanadium, titanium and boron, cooperate in eliminating the "hot shortness," and when used in the percentages shown, the finished tested product shows practically no cracks even after the flame test and Zyglo inspection.

In the test generally referred to as the "flame test," one end of the specimen is subjected to a torch for one minute, and thereafter a green fluorescent penetrant dye is applied and developed so as to disclose the presence of minute cracks, etc. Since such tests are well known, a detailed description herein is believed unnecessary and it is sufficient to say that under such rigorous tests the products treated in accordance with the present invention disclose very few, if any, perceptible cracks.

10 In the operation of the process, the austenitic stainless steel alloy is brought to a molten condition within the furnace and the ferro-compound of vanadium and titanium and the boron are added to the metal in the furnace or, if desired, to the ladle during tapping. Aluminum may be added in the deoxidizing procedure, in accordance with general furnace practice, and silicon may also be added for the maintenance of the physical properties and to promote fluidity. If desired, the aluminum and silicon may be added simultaneously with the 15 titanium, vanadium and boron, and the proportions of these will be the proportions usually added according to general furnace practice.

Specific examples of the process may be set out as follows:

25 *Example I*

A stainless steel alloy having the following analysis:

|              |     | Percent |
|--------------|-----|---------|
| Carbon       | max | 0.07    |
| 30 Manganese |     | 2.00    |
| Silicon      | max | 1.5     |
| Chromium     |     | 20.5    |
| Nickel       |     | 29.3    |
| Molybdenum   |     | 2.4     |
| 35 Copper    |     | 3.3     |

was heated in an electric furnace to molten condition, and to the molten metal just before tapping was added ferro vanadium and titanium in the proportions of 0.05% vanadium, 0.01% titanium, and 0.002% boron. The 40 casting test bars made from the alloy were subjected to the flame test and to the fluorescent dye penetrant (Zyglo) test, and it was found that there were practically no perceptible cracks, thus showing the elimination of hot shortness.

45 *Example II*

The operation was carried on as described in Example I, except that the vanadium was in the proportion of 0.25%, the titanium in the proportion of 0.15%, the 50 boron remaining at about 0.002%. The results obtained were comparable to those described in Example I.

*Example III*

55 The process was carried out as described in Example I except that the austenitic stainless steel had a different composition, containing 24% chromium, 20.5% nickel, 0.08% carbon, about 1.5% manganese, and 1.0% silicon. The procedure as described in Example I was 60 found to eliminate hot shortness in the above-described alloy.

*Example IV*

The process was carried out as described in Example I, except that the stainless steel alloy treated had about 65 17.65% chromium content, 13.65% nickel, 2.65% molybdenum, 0.08% carbon maximum, about 1.25% manganese, and about 1.0% silicon. Hot shortness was eliminated by the adding of the materials described in Example I.

*Example V*

The process was carried out as described in Example

IV, except that the stainless steel alloy treated had about 18.7% chromium and 10.5% nickel, the carbon, manganese, and silicon contents being the same as shown in Example IV. Comparable results were obtained.

*Example VI*

The process was carried out as described in Example IV except that the stainless steel alloy, which was otherwise the same, had a chromium content of 15% and a nickel content of 35%. The same results as described in Example IV were obtained.

In the treatment of austenitic cast stainless steels, the three added materials, namely, vanadium, titanium and boron, appear to produce together, as a total effect, the elimination of the hot shortness, and while the proportions of these may be varied within a substantially wide range depending upon the analysis of the particular austenitic cast stainless steel material being treated, the important new result of eliminating hot shortness is achieved by the use of all three materials.

Both corrosion-resistant and heat-resistant cast stainless steels are materially improved through the procedure of this invention. A distinction between the two steels is that the corrosion-resistant steels are generally used to resist attack at temperatures less than 1200° F., while heat-resistant alloys are generally used under conditions where the metal temperature is in excess of 1200° F. I have found that in the instance of both corrosion-resistant and heat-resistant stainless steel castings, a favorable cooperation between vanadium and titanium occurs to substantially eliminate hot shortness.

Exemplary of the practice of the invention in this connection are the following examples:

*Example VII*

A stainless steel alloy having the following analysis:

|            | Percent   |
|------------|-----------|
| Carbon     | max. 0.08 |
| Manganese  | 1.50      |
| Silicon    | 1.50      |
| Phosphorus | max. 0.04 |
| Sulphur    | max. 0.04 |
| Molybdenum | 2.0       |
| Chromium   | 18.0      |
| Nickel     | 9.0       |

was heated in an electric furnace to molten condition, and to the molten metal just before tapping was added ferro-vanadium and titanium in the proportions of 0.05% vanadium and 0.01% titanium. The casting test bars made from the alloy were subjected to the flame test and to the fluorescent dye penetrant (Zyglo), and it was found that there were practically no perceptible cracks, thus showing the elimination of hot shortness.

*Example VIII*

The operation was carried on as described in Example VII, except that the vanadium was in the proportion of 0.25%, and the titanium in the proportion of 0.15%. The results obtained were comparable to those described in Example VII.

*Example IX*

The process was carried out as described in Example VII, except that the austenitic stainless steel had a slightly different composition, containing 21% chromium and 12% nickel instead of the percentages set forth for these elements in Example VII. The procedure as described in Example VII was found to eliminate hot shortness in the above-described alloy.

*Example X*

The process was carried out as described in Example I, but with a stainless steel alloy having the following composition:

|            | Percent  |
|------------|----------|
| Carbon     | 0.20     |
| Manganese  | 2.0      |
| Silicon    | 2.0      |
| Phosphorus | 0.04     |
| Sulphur    | 0.04     |
| Chromium   | 24.0     |
| Nickel     | 18.0     |
| Molybdenum | max. 0.5 |

25 "Hot shortness" was eliminated by the adding of the material described in Example VII.

*Example XI*

The process was carried out as described in Example X except that the stainless steel alloy treated had 28% chromium and 22% nickel instead of the amounts of these elements specified in Example X. Comparable results were obtained.

30 While in the foregoing description I have set forth in detail specific steps and proportions for the purpose of illustrating preferred embodiments of the invention, it will be understood that such details of procedure, proportions, etc., may be varied widely by those skilled in the art without departing from the spirit of my invention.

I claim:

35 1. In a process for preventing "hot shortness" in an austenitic cast stainless steel alloy, the steps of heating the alloy to bring it to a molten state and then adding vanadium and titanium combined in a ferro-compound, the proportions of the vanadium being .05 to .25%, and of the titanium .01 to .15%.

2. In a process for preventing "hot shortness" in an austenitic cast stainless steel alloy, the steps of heating the alloy to bring it to a molten state and then adding to the molten alloy vanadium and titanium simultaneously, the proportion of the vanadium being .05 to .25%, and of the titanium .01 to .15%.

References Cited in the file of this patent

UNITED STATES PATENTS

|           |               |               |
|-----------|---------------|---------------|
| 1,542,232 | Girin         | June 16, 1925 |
| 2,432,617 | Franks et al. | Dec. 16, 1947 |
| 2,602,028 | Urban et al.  | July 1, 1952  |
| 2,750,283 | Loveless      | June 12, 1956 |
| 2,811,438 | Fink          | Oct. 29, 1957 |